

J. H. RICHARDS & B. BELLINGHAM.  
METHOD OF PRODUCING PISTON RINGS.  
APPLICATION FILED SEPT. 12, 1917.

1,278,015.

Patented Sept. 3, 1918.

Fig.1.



Fig.2.



Fig.3.

WITNESSES

Morris L. Sumner.

*John H. Richards*

INVENTORS

John H. Richards  
Benjamin Bellingham

by *James L. Morris,*  
*Attorney*

# UNITED STATES PATENT OFFICE.

JOHN HARTLAND RICHARDS AND BENJAMIN BELLINGHAM, OF SALTLEY, BIRMINGHAM, ENGLAND.

## METHOD OF PRODUCING PISTON-RINGS.

1,278,015.

Specification of Letters Patent. Patented Sept. 3, 1918.

Application filed September 12, 1917. Serial No. 180,963.

*To all whom it may concern:*

Be it known that we, JOHN HARTLAND RICHARDS and BENJAMIN BELLINGHAM, subjects of the King of Great Britain, residing at 5 Saltley, Birmingham, England, have invented certain new and useful Improvements in Methods of Producing Piston-Rings, of which the following is a specification.

This invention relates to piston rings for 10 packing the pistons of internal combustion, steam and other engines, pumps and the like, said rings being of that type which are provided upon their peripheries with a facing of anti-friction metal which makes contact with the cylinder wall, thus reducing 15 friction and wear to a minimum.

The object of the present invention is to apply the anti-friction metal to the iron or steel ring so that a true molecular cohesion 20 is attained between the said facing and the ring, thus allowing of free contraction and expansion of the ring without breaking or separation of the anti-friction facing, and the latter being secured to the ring solely by 25 its adhesion, without the use of dovetail interlocking parts or other special securing means.

The invention consists in first tinning 30 the peripheral surface of the ring, such tinning consisting in applying a flux to the said surface and then coating this surface with tin, the tin being melted by heat and spread over the surface by a hot iron or other appropriate means; and then applying 35 the anti-friction metal (which contains a proportion of tin) to the tinned surface by casting it thereon or by dipping the ring, the anti-friction metal being, by this means, fixed to the ring.

40 Figure 1 of the accompanying drawings is a section through a piston ring having an anti-friction facing in accordance with this invention.

Fig. 2 represents a transverse section 45 through the ring.

Fig. 3 shows a modification.

As shown in Figs. 1 and 2, the body part 50 of the piston ring consists of a split spring ring *a* made of cast iron or steel as usual, while applied to the outer surface or periphery of this cast iron or steel body is a layer or facing *b* of a suitable anti-friction or white metal (containing a proportion of tin) which thus bears against the walls of 55 the cylinder in which the piston works. In

order to apply this anti-friction coating, the peripheral surface is first coated with tin. This tinning operation consists in applying a flux to the surface and then a small quantity of tin is melted and spread over the said 60 surface by a hot iron or other appropriate means. After the surface of the ring has been thus tinned the anti-friction metal is cast on to it in a mold, or the anti-friction metal may be applied by successive dipping 65 operations, the ring being rotated so that its periphery moves within a bath of the molten metal, which adheres to the said periphery, the layer increasing in thickness with each successive rotation. Preferably a current of 70 cold air is arranged to play upon the deposited metal as it leaves the bath.

With either process the anti-friction metal is fixed to and is in molecular cohesion with the ring and is thus inseparable therefrom. 75

The anti-friction facing *b* is preferably reduced in thickness toward the ends of the ring.

As shown in Fig. 3, in addition to the anti-friction metal being applied to the periphery of the ring, as at *b*, it may also be applied to the lateral faces, as at *b*<sup>1</sup>, these faces having previously been prepared by tinning as above described. The friction between the lateral faces of the ring and the 85 sides of the groove in the piston is thus reduced.

Having fully described our invention, what we desire to claim and secure by Letters Patent is:—

1. A method of producing a piston ring 90 consisting in applying a flux to the peripheral surface of a split cast-iron or steel ring, spreading a thin coating of tin over the surface by the aid of heat, and applying to the 95 said tinned surface a layer of anti-friction metal containing tin while in a molten state so as to adhere to the said surface.

2. A method of producing a piston ring 100 consisting in applying a flux to the periphery and lateral faces of a split cast-iron or steel ring, spreading a thin coating of tin over the said faces by the aid of heat, and applying to the tinned surface a layer of anti-friction metal containing tin while in 105 a molten state so as to adhere to the said surface.

3. A method of producing a piston ring 110 consisting in applying a flux to the peripheral surface of a split cast-iron or steel ring,

spreading a thin coating of tin over the surface by the aid of heat, applying to the said tinned surface a layer of anti-friction metal containing tin, and reducing the thickness of said anti-friction coating at the free ends of the ring.

In testimony whereof we have hereunto

set our hands in presence of two subscribing witnesses.

JOHN HARTLAND RICHARDS.  
BENJAMIN BELLINGHAM.

Witnesses:

HENRY NORTON SKERRETT,  
H. O. PRATT.